

June 13, 1944.

A. W. HANSON

2,351,039

MAKING SIMULATED WOVEN FABRIC

Filed March 11, 1942



*Fig. 1*



*Fig. 2*



*Fig. 3*

INVENTOR.  
Alden W. Hanson  
BY

*Griswold & Burdick*  
ATTORNEYS

## UNITED STATES PATENT OFFICE

2,351,039

## MAKING SIMULATED WOVEN FABRIC

Alden W. Hanson, Midland, Mich., assignor to  
 The Dow Chemical Company, Midland, Mich.,  
 a corporation of Michigan

Application March 11, 1942, Serial No. 434,164

2 Claims. (Cl. 28—72)

This invention relates to an improved method of producing a simulated woven fabric.

It is old in the art to produce woven fabric by means of looms wherein a single filament called the woof or filler carried by a shuttle traverses a series of warp filaments going over and under alternate single warp filaments or alternate pairs of warp filaments, each traverse of the width of the fabric by the shuttle being known as a "pick." This method of producing woven fabric is relatively slow, since the shuttle must traverse the entire width of the fabric to increase the fabric length by approximately the width of a single filament.

It is, therefore, an object of the present invention to provide a method of producing fabric indistinguishable from that made by weaving, at a faster rate and more economically than can be produced by weaving.

The simulated woven fabric is produced by braiding filaments to make a tube on a standard tube braiding machine and thereafter slitting the tube in a manner to be more fully described hereinafter. It is pointed out that in the specification and appended claims the term "simulated woven fabric" is intended to include flat articles narrow enough to be described ordinarily as tapes or ribbons as well as those articles having sufficient width to be included under the commonly used definition of the term "fabric."

The present invention comprises braiding a tube in which the filaments cross at an angle of substantially 90° to each other from filamentous material on a standard tube braiding machine and subsequently slitting the thus-produced braided tube along the path of one filament in the tube. In slitting a normally braided tube the slit is helical in direction along the longitudinal axis of the tube. When the tube is slit in this manner from end to end throughout its length, or if it is slit thus throughout a part of its length and the slit portion severed from the tube, a fabric will be produced which is substantially identical with that produced by simple weaving on a loom. The width of the fabric that may be produced in this manner is dependent upon the diameter of the braided tube from which it is produced.

If desired, the so-formed fabric may be passed between rolls or pressed between plates or otherwise treated to remove the curl from the helix and produce a flat fabric. In the case of fabrics prepared from filaments made of thermoplastic materials a convenient method of removing the curl from the helix is to pass the fabric between heated rolls which at the same time exert a slight pressure on the fabric. Fabrics prepared according to the method of the present invention from thermoplastic filaments may be prevented from fraying or unraveling along the cut edges

by pressing the edges of the fabric between heated plates or rolls in such a manner as to cause the loose ends of the filaments to fuse or stick together under the combined effect of heat and pressure. Other suitable means may be employed to bind the loose ends of the filaments, according to the particular material from which the fabric is made.

It is apparent that the filaments which are braided to form fabric by the method of the present invention need not be of textile fibers alone but that they may be composed of synthetic resinous materials such as vinylidene chloride polymers and copolymers, cellulose derivatives, metals, or any suitable material which can be formed into threads, filaments, narrow bands, and the like. The braided fabric may be composed of like filaments or of dissimilar filaments such as for example, partly of filaments of synthetic resinous materials, and partly of wire, or of wire coated with cellulose derivatives or of other materials. For most purposes it is an advantage to use filaments composed of the same materials, but it is apparent that filaments composed of different materials can be used, when desired, and that it may be of advantage to employ filaments made of different materials to produce fabric having a special effect or for a particular use.

For purposes of illustration and a better understanding of the method of the present invention reference is now had to the drawing wherein:

Figure 1 shows in diagrammatic form a portion of an open mesh braided tube;

Figure 2 illustrates the method of helically slitting the braided tube along the path of one filament; and,

Figure 3 shows a portion of the fabric after it has been pressed to remove the curl from the helix.

The method of the present invention is particularly useful for rapidly and economically producing a simulated woven fabric from threads, filaments, narrow bands, tapes or ribbons. Thus, synthetic monofil having a diameter of 0.011 inch can be woven to form fabric having 16 monofil to the inch on a standard loom at the rate of only about 1.5 square feet per minute. Using a tube braiding machine having 800 carriers, a tube in which the monofil cross at an angle of 90° to each other can be braided from like monofil which, when slit helically as previously described, will produce similar fabric having 16 monofil to the inch at the rate of about 3 square feet per minute.

It also has been found that the method of the present invention is especially suited for producing open mesh fabric from monofil or threads and more particularly for producing simulated woven fabric suitable for screens, sieves, bolting cloth, nets, and the like.

The method of the present invention also is of advantage for producing close woven fabric from narrow bands, tapes or ribbons. Relatively large spools of such filaments can readily be placed without difficulty on the carriers of a standard braiding machine whereas special bobbins and shuttles would be required to weave such filaments on a standard loom. Fabric produced from narrow bands or ribbons made of synthetic resinous materials are particularly suited for covering chair seats.

The following examples illustrate the practice of the invention but are not to be construed as limiting the scope thereof.

*Example 1*

Filaments 0.020 inch in diameter were prepared from a composition comprising a copolymer consisting of about 90 per cent vinylidene chloride and correspondingly about 10 per cent vinyl chloride, plasticized with 7 per cent by weight of di-(alpha-phenylethyl) ether, based on the weight of the composition. The filaments were wound on bobbins of a standard 96-carrier tube braiding machine. The braiding machine was adjusted to braid an open mesh tube 1.35 inches in diameter composed of filaments laid down at an angle of 45° to the longitudinal axis of the tube, and were spaced equally apart and numbered approximately 16 filaments per inch when measured at right angles to one set of parallel filaments. The tube could be produced at a rate of 1.06 feet of tube length per minute or 63.6 linear feet of tube per hour. The braided tube was slit helically throughout its length along the path of one of the filaments. The thus-produced helix was pressed by passing it between nickel-plated rolls heated to a temperature of 125° C. There was produced a flat fabric 3 inches wide and 90 feet long. This corresponds to approximately 22.5 square feet of fabric. The fabric was substantially identical with that obtained by weaving like filaments into a similar open mesh fabric on a loom.

*Example 2*

Using like filaments to those described in Example 1 an 800 carrier tube braiding machine can be used to braid a tube 11.2 inches in diameter, in which the filaments cross at an angle of 90° to each other and are spaced equally apart and number 16 filaments per inch. The tube can be braided at the rate of 1.06 linear feet per minute or 63.6 feet per hour. When slit along the path of one filament a sheet of fabric about 24.8 inches wide and 90 feet long is produced. This corresponds to about 180 square feet of fabric per hour as compared to about 90 square feet of fabric per hour that can be produced by weaving on a standard loom.

*Example 3*

In a manner similar to that described in Example 1 and using filaments having a diameter of 0.020 inch a 3000 carrier tube braiding machine can be used to braid a tube 42.2 inches in diameter in which the filaments cross at an angle of 90° to each other. The tube can be braided at a rate of 1.06 linear feet per minute or 63.6 feet per hour. When slit helically along one filament there is produced a sheet of fabric 93.5 inches wide and 90 feet long. This corresponds to a rate of production of about 700

square feet of fabric per hour. This is approximately eight times as fast as fabric can be produced by weaving like filaments on a loom.

5

*Example 4*

Narrow bands 0.125 inch wide and 0.020 inch thick, prepared from the composition described in Example 1, were wound on bobbins of a 96 carrier tube braiding machine. The machine was adjusted to braid a tube in which the bands were laid down flat and crossed at an angle of 90° to each other. The narrow bands were spaced close together and numbered 8 per inch when measured at right angles to one series of bands. The tube had a diameter of 2.7 inches and could be braided at the rate of 2.1 linear feet per minute or 126 feet per hour. When slit helically throughout its length along the path of one band and pressed to remove curl from the helix, there was produced a fabric 6 inches wide and 178 feet long. This corresponds to 89 square feet of fabric. The fabric was suitable for covering chair seats.

10 20 25 30 35 40 45 50 55 60 65 70 75 80 85 90 95

The above examples clearly show that simulated woven fabric having a simple weave can be produced by the method of the present invention at a rate substantially faster than fabric can be produced by weaving like filamentous material on a loom.

The rate at which simulated woven fabric can be produced by the method of the present invention will vary depending upon the number of carriers on the braiding machine, the size and shape of the filaments or threads being braided, and the number of filaments per inch of fabric.

While the invention has been described with particular reference to certain embodiments utilizing vinylidene chloride copolymeric filaments and a standard tubular braiding machine, it is not intended that the scope of the invention be limited thereto. It is apparent that the method may be equally as well applied to produce fabric from monofils of any suitable shape or from threads, tapes or narrow bands consisting of a plurality of monofils spun or woven together. It is understood that the invention is susceptible of variations and that the invention is not to be construed as limiting except as defined by the following claims.

I therefore particularly point out and distinctly claim as my invention:

1. The method of producing a simulated woven fabric at a faster rate than can be obtained by weaving on a loom which comprises braiding a tube of filaments in which the filaments cross at an angle to each other and slitting said braided tube parallel to the path of one filament in a helical direction along the longitudinal axis of the braided tube.

2. The method of producing a simulated woven fabric at a faster rate than can be obtained by weaving on a loom which comprises braiding a tube of filaments in which the filaments cross at an angle substantially 90° to each other, slitting said braided tube parallel to the path of one filament in a helical direction along the longitudinal axis of the braided tube, and pressing the thus-formed fabric to remove the curl from the helix and form a flat fabric, said fabric being substantially identical with that produced by simple weaving on a loom.

ALDEN W. HANSON.